

Patented Oct. 27, 1925.

1,558,853

# UNITED STATES PATENT OFFICE.

ALPHONSE FLORENT EIJSSEN, OF HEERLEN, NETHERLANDS.

PROCESS FOR THE METALLIZATION OF PORCELAIN OR GLASS.

No Drawing.

Application filed December 12, 1924. Serial No. 755,580.

To all whom it may concern:

Be it known that I, ALPHONSE FLORENT EIJSSEN, a subject of the Queen of Holland, residing at Heerlen, Province of Limburg, 5 Kingdom of the Netherlands, have invented an Improved Process for the Metallization of Porcelain or Glass, of which the following is a specification.

The invention relates to a process for rendering objects of porcelain or glass conducting, in order to deposit metals thereon according to a galvanic method.

It is known to render an object conducting by covering it with a thin layer of silver. 15 To this end the object is first provided with a coating of alkali silicate and then with a coating containing  $KCN$ ,  $NH_4Fl$  and  $AgCl$ . This coating is reduced with hydrazine, the reduction of the silver being completed by 20 brushing with a metal brush (of copper, brass, iron, zinc, etc.).

According to the invention in order to obtain a metallized conducting surface without using a silver salt, glycerol is rubbed 25 with a brush of brass or similar material on to the surface of the object to be metallized, by which treatment a deposit of brass is obtained on the porcelain or glass, which is made conducting in this manner. A little 30 nitrate of silver may be added to the glycerol when silver is desired in the deposit. Generally however this is not required. In lieu of glycerol also other viscous polyvalent alcohols may be used such as glycol and 35 the like.

In order to cover such a metallized surface with more metal, it is connected by 40 means of a copper wire to the negative pole of a dynamo or a galvanic battery, the positive pole of which is connected to a copper plate which is placed with the object to be metallized in a solution of e. g.

1 liter water.

200 grams sulphate of copper.

45 20 grams sulphuric acid of 66° Bé.

Then an electric current is passed of a density of about 5 amperes per square decimeter of the surface to be metallized.

For applying the invention, the surface to 50 be treated must first be dulled, e. g. by means of a sand blast machine working at a pressure of  $\frac{1}{2}$  kg. per sq. cm. and fine white sand. The dulled surface is rubbed with a very small quantity of glycerol using 55 a brass brush. It will be observed immediately that a very adherent deposit of brass

is obtained on the porcelain or glass, and care must be taken to rub the dulled glass with the brass brush until the surface is quite dry so that it has a dark green appearance. If too much glycerol is used good adhesion of the metal to the treated object cannot be obtained.

After this treatment, the rubbed surface of the object has wrapped round it or applied to it by a copper wire which is connected to the negative pole of a source of current, the positive pole of which is connected to a copper plate immersed in the same bath as the object to be metallized, 60 said bath being filled with a solution of copper sulphate of about the above mentioned composition. The bath is electrolyzed at a temperature of 14-20° C. and a current density of 5 amp. per square decimeter of 65 the rubbed surface. After a few minutes it is observed that the rubbed part is covered with a layer of copper. When the objects are metallized sufficiently, they are removed 70 from the bath and polished.

They may be afterwards covered with 75 silver or nickel in the usual way.

In the manner described one may e. g. metallize the outside of porcelain kettles. Such kettles have the advantage that they 80 do not burst, are less subject to breakage and remain hot for a longer period than ordinary porcelain kettles. Porcelain cans for coffee, tea or milk may be treated according to the invention to protect them 85 against breakage. Such metallized objects of glass or porcelain compared with similar metal objects have the advantage that they do not leave a metal taste when in use and can be cleaned very easily. They have therefore 90 hygienic advantages. It is also possible to use the invention for ornamental purposes.

What I claim is:

1. A process for metallizing a dull surface of non-conducting hard material comprising rubbing the surface with a very small quantity of a viscous polyvalent alcohol by means of a metal brush and then depositing electrolytically a further metal 105 coating.

2. In a process for metallizing a dull surface of non-conducting hard material the step of rubbing the surface with a very small quantity of glycerol by means of a 110 metal brush.

3. In a process for metallizing a dull sur-

face of non-conducting hard material the step of rubbing the surface with a very small quantity of glycerol by means of a brass brush.

5. A process according to claim 3 in which nitrate of silver is added to the glycerol.

5. A process for metallizing objects of unglazed porcelain comprising rubbing the surface to be metallized with a very small

quantity of glycerol by means of a brass 10 brush, connecting the object by means of a copper wire to the negative pole of an electric machine while the object is immersed in an electrolytic bath containing a solution of the metal to be deposited.

15

In testimony whereof I affix my signature.

ALPHONSE FLORENT EIJSSEN.